

Dec. 17, 1946.

E. C. PFEFFER, JR., ET AL

2,412,832

TEXTILE MATERIAL AND METHOD OF PREPARING IT

Filed Oct. 30, 1943

STABILIZATION DATA

Shrinkage in 5 Washes After Stabilizing Process:

Formulas on Percent by Weight Basis

| Fabric Construction                                                                                                                                         | Scouring Loss    | (A)<br>Shrinkage of<br>Untreated<br>Fabrics (in<br>5 Washes) | (B)<br>%<br>%1-5 | (1)<br>Glycol;<br>.25% Oxalic<br>Acid | (2)<br>Glycol;<br>.25% Oxalic<br>Acid;<br>3.36% P-64 | (3)<br>Urea-Form.<br>(Rhonite 609);<br>.1% NH <sub>4</sub> Cl |
|-------------------------------------------------------------------------------------------------------------------------------------------------------------|------------------|--------------------------------------------------------------|------------------|---------------------------------------|------------------------------------------------------|---------------------------------------------------------------|
| 75% Viscose Staple &<br>25% Acetate Staple, Blended<br>Plain Weave<br>18/1 28 T-Z<br>warp and filling<br>50x50 Count<br>4.8 oz/yd                           | 1.28"/yd<br>3.6% | 14.9                                                         | 2.4              | 6.9 .8                                | 5.0 .6                                               | 6.9 .8                                                        |
| 85% Viscose Staple &<br>15% Aralac, Blended<br>Plain Weave<br>21/1 16 T-Z<br>warp and filling<br>69x55 Count<br>4.7 oz/yd                                   | .56"/yd<br>1.6%  | 11.8                                                         | .9               | 8.9 1.1                               | 2.8 .6                                               | 5.0 0                                                         |
| 50% Viscose Staple &<br>50% Acetate Staple, Blended<br>Cavalry Twill Weave<br>18/1 19 T-S warp<br>18/1 17 T-Z filling<br>10.1x67 Count<br>8.1 oz/yd         | 1.76"/yd<br>4.9% | 12.4                                                         | 2.2              | 7.2 .6                                | 2.8 .8                                               | 5.3 0                                                         |
| 80% Viscose Staple &<br>20% Acetate Staple, Blended<br>2x1 Twill Weave<br>24/1 19 T-S warp<br>24/1 19 T-Z filling<br>116x66 Count<br>6.5 oz/yd              | 2.32"/yd<br>6.4% | 13.5                                                         | 1.1              | 6.1 .6                                | 3.9 0                                                | 5.3 .3                                                        |
| 60% Viscose Staple &<br>40% Acetate Staple, Blended<br>Plain Weave<br>30/2 19 T-Z singles<br>13 T-S ply<br>warp and filling<br>65x68 Count<br>6.5 oz/yd     | 2.25"/yd<br>6.2% | 11.7                                                         | 1.9              | 3.9 .3                                | 2.2 .3                                               | 3.3 0                                                         |
| 70% Viscose Staple &<br>30% Acetate Staple, Blended<br>2x2 Twill Weave<br>20/2 15 T-Z singles<br>8 T-S ply,<br>warp and filling<br>56x71 Count<br>8.8 oz/yd | .96"/yd<br>2.7%  | 11.0                                                         | 4.8              | 3.1 .8                                | .8 .8                                                | 2.8 .8                                                        |
| 100% Filament Rayon<br>(Viscose)<br>98 denier warp<br>152 denier filling<br>92x70 Count<br>2.7 oz/yd                                                        | .1"/yd<br>.3%    | 9.2                                                          | 1.3              | 1.9 .3                                | .8 0                                                 | 2.2 .3                                                        |

Inventors  
Edward C. Pfeffer, Jr.  
Jack E. Elberg,  
by Robert C. [Signature]  
Attys.

## UNITED STATES PATENT OFFICE

2,412,832

TEXTILE MATERIAL AND METHOD OF  
PREPARING IT

Edward C. Pfeffer, Jr., and Jack Epelberg, Troy,  
N. Y., assignors to Cluett, Peabody & Co., Inc.,  
Troy, N. Y., a corporation of New York

Application October 30, 1943, Serial No. 508,368

8 Claims. (Cl. 8—115.6)

1

This invention pertains to textiles and relates more particularly to a novel textile material, for example a woven fabric permanently stable with respect to laundry shrinkage and resistant to wrinkling, crushing and creasing, and if desired of a soft hand and good draping quality, and to a novel method of preparing such a material, the present invention representing a further development of an improvement upon the invention disclosed in the copending application of Pfeffer and Epelberg, Serial No. 495,620, filed July 21, 1943.

The term "textile material" as herein employed is intended to include filaments, fibers, staple or yarns, whether in the finished state or at some intermediate stage in the production thereof. The term also includes fabrics whether knitted, woven or felted, as well as garments or other articles made from such fabrics.

A principal object of the present invention is to provide textile material, for instance of any of the classes just above enumerated—for more specific example a woven fabric—which possesses even better stability with respect to dimensional shrinkage, together with equal or better resistance to crushing than the material disclosed in the aforesaid application as well as other advantages of the latter material and which, if desired, may have a very soft hand and fine draping qualities. A further object is to provide a novel method of preparing textile material of this improved character. Other and further objects and advantages of the invention will be pointed out in the following more detailed description and by reference to the annexed drawing which consists of a table showing the characteristics of the fabric of the present invention as compared with those of untreated fabric and of fabric which has been treated in accordance with the procedure of the aforesaid application.

In the above application it was pointed out that customary previous modes of stabilizing and crushproofing textile materials had involved the use of solutions or suspensions of intermediate condensation products of synthetic resins or resin components either with or without a plasticizer, and forming and curing the resin in situ, and that such resinous substances as had commonly been employed (phenol formaldehyde, urea formaldehyde, and melamine formaldehyde, etc.)

2

when used alone possess many disadvantages which substantially lessen their field of usefulness. For example, some of them have or emit during curing an exceedingly disagreeable odor or irritating or toxic fumes necessitating special and extensive precautions in their use; in some instances the disagreeable odor is persistent in or develops in the fabric after finishing; some of these resinous type materials cause permanent discoloration or browning of the fabric so that they are not applicable to white material; some of them make the constituent fibers of the fabric tender thereby reducing the tensile strength of the fabric; and some of them are unduly expensive, particularly when employed in the large amounts sufficient effectively to provide crease resistance as well as dimensional stability.

The aforesaid application further disclosed, as a wholly novel concept, the employment of a dialdehyde, glyoxal



also known as oxalic aldehyde, or ethanedial as a stabilizing and crushproofing medium in substitution for the formaldehyde theretofore employed, and pointed out substantial advantages for the glyoxal as compared with the materials which had previously been employed, for example the fact that the glyoxal may be or in fact must be used in low concentrations, for example from 0.6% to 4.65% by weight in the treating bath, whereas such prior materials as urea formaldehyde condensation products must be used in concentrations of from 6% to 8% for stabilization and from 14% to 16% for creaseproofing.

Further, it was noted that glyoxal does not emit disagreeable fumes during curing; it does not substantially tender the textile material or make it brittle, when used in the concentrations requisite for stabilization or crushproofing; it does not discolor or brown the textile material to any harmful degree; it may readily be applied without necessitating special equipment, and it has little odor in solution of a strength suitable for its intended use.

It was also noted that the glyoxal is applied to the fabric in water solution but it does not exist as the above compound when in water solution since it hydrates to form a compound known

as tetrahydroxydioxane, which has the following structural formula:



When the water in which this material is dissolved is evaporated and further heat is applied, the material readily dehydrates yielding glyoxal as shown by the following formula:



While we do not definitely know the exact action which occurs when cellulose in association with glyoxal is heated, we believe that a reaction takes place in consequence of which the cellulose of the individual fibers of the fabric is at least partially converted into a reaction product which may be termed "dicellulose diacetal" or "cellulose glyoxal," as may be preferred, such product being of the long-chain, high molecular weight type, but with cross-linkages making it more stable than the formaldehyde resins.

We have now discovered that whereas glyoxal alone (or in association with a catalyst accelerator) in these low concentrations provides a degree of stabilization and crushproofing comparable with the results obtained by the use of larger amounts of the formaldehyde condensation products previously employed, unexpectedly better results are obtainable by associating with the glyoxal one or more amino-aldehyde water-dispersible resinous condensation products, for example urea or melamine formaldehyde, but employing such resinous condensation products in amounts far too small (except in association with the glyoxal) to accomplish either stabilization or crushproofing. Further, wholly unexpectedly it has been discovered that when thus used in association, the stabilizing effect of the combined resin and glyoxal is even greater than that of the equivalent amount of either material alone and that damage to the fabric is less than might result from an equivalent amount of either the glyoxal or the resin condensation product by itself.

For certain purposes, for instance in the manufacture of men's sport shirts, it is desirable that the fabric be very soft and possess excellent draping qualities or in other words that it should have a very "soft hand," although this characteristic is not normally possessed by most fabrics made from synthetic fibers. It has further been discovered that when the glyoxal and resin are thus used in association, as above suggested, a very soft hand or feel may be imparted to the fabric by including in the treating bath a cation-active softener, for example one of the quaternary ammonium compounds.

As described in the aforesaid application, it is found desirable, in order to hasten the action and to avoid overheating of certain types of fabric, to employ an acid catalyst to facilitate the reaction between the glyoxal and the cellulose of the fiber. Among such catalysts may be mentioned oxalic acid, ammonium chloride, ammonium sulphate, and ammonium nitrate. Oxalic acid is highly satisfactory since its use avoids the development of any substantial color during heat treatment.

As illustrative, without limitation of the scope of the invention, the following suggestions as to reagent strengths and conditions of treatment are cited, it being noted that in accordance with the present invention substantially the same amount of glyoxal and catalyst are employed as disclosed in the above application, the resinous material being in addition thereto.

1. Amount of glyoxal:

15 to 120 cubic cms. of 30% glyoxal solution per liter of treating bath, or approximately .6 to 4.65% glyoxal by weight in the treating bath.

2. Type of catalyst:

Acid-reacting, such as organic acids or salts of inorganic acids or organic acids which produce an acid effect.

3. Amount of catalyst:

1/8 to 4 gms. per liter of treating bath, or approximately .0125 to .40% by weight of treating bath.

4. Amount of resin:

12 to 50 gms. of 100% condensation product per liter of treating bath or approximately 1 to 5% by weight of the treating bath.

5. Amount of softener, if used:

Approximately 1% by weight of treating bath.

6. Baking temperature:

212° F. to 350° F.

7. Baking time:

2 minutes to 40 minutes.

Obviously the baking temperature and the baking time are inversely related.

Certain condensation products (now obtainable from the Reichhold Chemicals, Inc., and from the American Cyanamid Company, respectively) which are useful in the practice of the present invention but which as yet have no established chemical names, are herein for convenience referred to as "Beckamine P-364" and "Aerotex M-3," and are herein identified and defined respectively as follows:

Beckamine P-364 is a water-dispersible condensation product of urea formaldehyde. Its preparation is fully described in copending application Serial No. 540,883, filed June 17, 1944, and assigned to Reichhold Chemicals, Inc., Boston, Massachusetts, from which this reagent may be obtained.

Aerotex M-3 is a methylated methylol-melamine and may be prepared substantially as follows:

Formula.—960 parts by weight of formalin (37% by weight  $\text{CH}_2\text{O}$ ) and 252 parts by weight of melamine are charged into a reaction vessel fitted with an agitator, thermometer, and reflux condenser and arranged so that it can be placed under a vacuum and heated. The contents of the reaction vessel are heated for one-half hour to a temperature of 62° C. and the pH adjusted to 7.5 with 2 normal NaOH. After heating for another one-half hour, a vacuum of 28 inches of mercury is applied and the mixture concentrated by removal of water. After 40 minutes' heating at approximately 54° C. the heat and vacuum are removed and there is added 1000 parts by weight of methyl alcohol containing enough 2 normal  $\text{H}_3\text{PO}_4$  to neutralize the 2 normal NaOH added previously. The mixture at a pH of 6.4 is then heated to distill off an azeotropic mixture of methanol and water, anhydrous methanol being continuously added to replace the distillate. After heating in this way for

about 6 to 7 hours, one part of the distillate will tolerate 100 parts of toluol and the resin is considered dried. It is then concentrated under a vacuum of 28 inches of mercury to a solids content of approximately 50%. The methylated methylol-melamine thus prepared may be dispersed in water to a concentration of 10% resin solids.

Hereinafter, when Beckamine P-364 and Aerotex M-3 are referred to, it is understood that these terms designate the products above described respectively, or the equivalents thereof.

The following special examples are given as illustrative of the application of the present novel process as a practical matter in materials of different types.

#### EXAMPLE 1

A plain weave, 100% spun viscose rayon fabric in the greige, made of 28/1 warp and 14/1 filling yarns of spun viscose rayon staple fiber is desized, scoured and dried on the tenter frame. The white, pure finished fabric has a count of 66 x 41 and a weight of 4 oz. per yard. This fabric is then passed through an impregnating solution containing 60 cubic centimeters of glyoxal solution (of 30.2% glyoxal content by weight), 3 grams of oxalic acid, and 45 grams of a water dispersible condensation product of urea formaldehyde (produced by Reichhold Chemicals Inc. and designated as P-364 Beckamine) per liter of solution. This urea formaldehyde product is condensed to a molecular weight such that it is completely dispersible in water in a very finely divided state, but is not sufficiently soluble to produce a clear solution. On a weight percentage basis this solution contains 2.25% glyoxal, 0.296% oxalic acid, and 3.36% urea formaldehyde reaction product by weight. After the fabric is passed through this solution and is well wetted out, it is squeezed to remove excess solution and is then dried on a tenter frame in air at around 180° F. to dimensions before impregnating. The dried fabric is then cured in a tenter oven or loop dryer oven in circulating air at 280° F. for 8 minutes, after which it is soaped, rinsed, and dried to the original pure finish fabric dimensions on a tenter frame. The resulting fabric is white, free from any odor, firm and resilient, with greatly improved resistance to shrinkage on washing, which effect is permanent to washing, and has improved resistance to creasing and crushing. A comparison of these properties of the untreated pure finish fabric and of the treated fabric is shown below. The tensile strength and abrasion resistance of the fabric are not appreciably affected by the process.

#### Shrinkage on washing, inches per yard

[5 modified rayon washes—mild soap solution at 100°-120° F. for 30 min.]

| Washes.....    | Warp<br>1 | Warp<br>2 | Warp<br>3 | Warp<br>4 | Warp<br>5 |
|----------------|-----------|-----------|-----------|-----------|-----------|
| Untreated..... | 3.5       | 3.9       | 4.43      | 4.26      | 4.20      |
| Treated.....   | 0         | .1        | .1        | .2        | .1        |

<sup>1</sup> Denotes a gain.

#### Shrinkage on washing, inches per yard

[5 modified rayon washes—mild soap solution at 100°-120° F. for 30 min.]

|                | Warp | Filling | Warp | Filling | Warp | Filling | Warp | Filling | Warp | Filling |
|----------------|------|---------|------|---------|------|---------|------|---------|------|---------|
| Washes.....    | 1    |         | 2    |         | 3    |         | 4    |         | 5    |         |
| Untreated..... | 6.10 | 1.27    | 6.53 | 1.50    | 7.13 | 1.47    | 7.03 | 1.30    | 7.23 | 1.27    |
| Treated.....   | 0    | .1      | 0.2  | .1      | .1   | .2      | .1   | .2      | .1   | .2      |

The process loss is 1.3 inches per yard in the warp, none in the filling.

#### Crease resistance

[Percentage recovery in one min. from a 180° fold formed under standard conditions]

|                | Per cent |
|----------------|----------|
| Untreated..... | 45       |
| Treated.....   | 85       |

The process loss is .9 inch per yard in the warp.

#### Crease resistance

[Percentage recovery in one min. from a 180° fold formed under standard conditions]

|                | Per cent |
|----------------|----------|
| Untreated..... | 70       |
| Treated.....   | 80       |

7  
EXAMPLE 3

A 2 x 2 twill, 70% spun viscose rayon and 30% spun acetate rayon fabric in the greige, made of blended 20/2—15 Z turns in the singles and 8 S turns in the ply in both warp and filling yarns is desized, scoured and dried on the tenter frame. The loss on the above operation is 0.96 inch per yard corresponding to 2.7%. The white, pure finished fabric has a count of 56 x 47, and a weight of 8.8 oz. per yard. This fabric is then passed through an impregnating solution containing 60 cubic centimeters of glyoxal solution (of 30.2% glyoxal content by weight), 3 grams of oxalic acid and 40 cubic centimeters of a water-soluble, thermosetting alkyl urea formaldehyde condensation product (manufactured by Sharples Chemicals Company) per liter of solution. On a weight percentage basis this solution contains 2.25% glyoxal, .296% oxalic acid and 1.95% alkyl urea formaldehyde reaction product by weight. After the fabric is passed through this solution and is well wetted out, it is squeezed to remove excess solution and is then dried on a tenter frame in air at around 180° F. to dimensions before impregnating. The dried fabric is then cured in a tenter oven or loop dryer oven in circulating air at 280° F. for 8 minutes, after which it is soaped, rinsed and dried to the original pure finish fabric dimensions on a tenter frame. The resulting fabric is white, free from any odor, firm and resilient, with greatly improved resistance to shrinkage on washing, which effect is permanent to washing, and has improved resistance to creasing and crushing. A comparison of these properties of the untreated pure finish fabric and of the treated fabric is shown below. The tensile strength and abrasion resistance of the fabric are not appreciably affected by the process.

## Shrinkage on washing, inches per yard

[5 modified rayon washes—mild soap solution at 100°-120° F. for 30 min.]

| Washes.....    | Warp | Filling | Warp | Filling | Warp | Filling | Warp | Filling | Warp | Filling |
|----------------|------|---------|------|---------|------|---------|------|---------|------|---------|
|                |      |         |      |         |      |         |      |         |      |         |
| Untreated..... | 2.25 | .3      | 2.77 | .26     | 3.55 | .46     | 3.6  | .56     | 3.97 | .66     |
| Treated.....   | .1   | .1      | .1   | 0       | 0    | 0       | .2   | .1      | .2   | 0       |

The process loss is .8 inch per yard in the warp, and .5 inch per yard in the filling.

## Crease resistance

[Percentage recovery in one min. from a 180° fold formed under standard conditions]

|                | Per cent |
|----------------|----------|
| Untreated..... | 80       |
| Treated.....   | 90       |

## EXAMPLE 4

A 100% plain woven filament viscose rayon fabric made of 98 denier warp and 152 denier filling yarns, with a count of 92 x 70 and weighing 2.7 oz. per yard is desized, scoured and dried on the tenter frame. The loss in the above operation is .1 inch per yard corresponding to .3%. The white, pure finished fabric is passed through an impregnating solution containing 60 cubic centimeters of glyoxal solution (of 30.2% glyoxal content by weight), 3 grams of oxalic acid, and 38 grams of a water-soluble condensation product of melamine formaldehyde (produced by American Cyanamid Company and designated as Aerotex M3) per liter of solution. On a weight percentage basis this solution contains 2.25% gly-

oxal, 2.96% oxalic acid and 3.0% Aerotex M3 by weight. After the fabric is passed through this solution and is well wetted out, it is squeezed to remove excess solution and is then dried on a tenter frame in air at around 180° F. to dimensions before impregnating. The dried fabric is then cured in a tenter oven or loop dryer oven in circulating air at 280° F. for 8 minutes, after which it is soaped, rinsed and dried to the original pure finish fabric dimensions on a tenter frame. The resulting fabric is white, free from odor, firm and resilient, with greatly improved resistance to shrinkage on washing, which effect is permanent to washing, and has improved resistance to creasing and crushing. A comparison of these properties of the untreated, pure finish fabric and of the treated fabric is shown below. The filling shrinkage is always much lower in the untreated fabric, and is also satisfactorily controlled. The tensile strength and abrasion resistance of the fabric are not appreciably affected by the process.

## Shrinkage on washing, inches per yard

[5 modified rayon washes—mild soap solution at 100°-120° F. for 30 min.]

| Washes.....    | Warp 1 | Warp 2 | Warp 3 | Warp 4 | Warp 5 |
|----------------|--------|--------|--------|--------|--------|
| Untreated..... | 2.83   | 3.06   | 3.1    | 3.2    | 3.3    |
| Treated.....   | 0      | .3     | .1     | .3     | .2     |

The process loss is .6 inch per yard in the warp.

## Crease resistance

[Percentage recovery in one minute from a 180° fold formed under standard conditions]

|                | Per cent |
|----------------|----------|
| Untreated..... | 45       |
| Treated.....   | 60       |

## EXAMPLE 5

A plain weave, 85% spun viscose rayon and 15% Aralac (casein fiber) fabric in the greige made of blended 21/1—16 Z turns in the singles in both warp and filling yarns, is desized, scoured and dried on a tenter frame. The loss in the above operation is 0.56 inch per yard corresponding to 1.6%. The white, pure finished fabric has a count of 69 x 55 and a weight of 4.7 oz. per yard. This fabric is then passed through an impregnating solution containing 60 cubic centimeters of glyoxal solution (of 30.2% glyoxal content by weight), 3 grams of oxalic acid, 30 grams of the water-dispersible urea formaldehyde condensation product designated as P-364 Beckamine and 20 grams of the water-soluble melamine formaldehyde reaction product known as Aerotex M3, per liter of solution. On a weight percentage basis this solution contains 2.25% glyoxal, .296% oxalic acid, 2.24% P-364 Beckamine and 1.56% Aerotex M3 by weight. After the fabric is passed through this solution and is well wetted out, it is squeezed to remove excess solution and is then dried on a tenter frame in air at around 180° F. to dimensions before impregnating.

## 9

ing. The dried fabric is then cured in a tenter oven or loop dryer oven in circulating air at 280° F. for 8 minutes, after which it is soaped, rinsed, and dried to the original pure finish fabric dimensions on a tenter frame. The resulting fabric is white, free from odor, firm and resilient, with greatly improved resistance to shrinkage on washing, which effect is permanent to washing, and has improved resistance to creasing and crushing. A comparison of these properties of the untreated pure finish fabric and of the treated fabric is shown below. The table shows only the warp shrinkage. The filling shrinkage is always much lower in the untreated fabric, and is also satisfactorily controlled. The tensile strength and abrasion resistance of the fabric are not appreciably affected by the process.

*Shrinkage on washing, inches per yard*

[5 modified rayon washes—mild soap solution at 100°-120° F. for 30 min.]

| Washes.....    | Warp 1 | Warp 2 | Warp 3 | Warp 4 | Warp 5 |
|----------------|--------|--------|--------|--------|--------|
| Untreated..... | 3.9    | 4.06   | 4.06   | 4.03   | 4.23   |
| Treated.....   | 0      | .1     | .3     | .3     | .3     |

The process loss is 1.3 inches per yard in the warp.

*Crease resistance*

[Percentage recovery in one min. from a 180° fold formed under standard conditions]

|                 | Per cent |
|-----------------|----------|
| Untreated ..... | 50       |
| Treated .....   | 80       |

## EXAMPLE 6

A plain weave, 100% spun viscose rayon fabric in the greige, made of 28/1 warp and 14/1 filling yarns of spun rayon viscose rayon staple fiber is desized, scoured, and dried on a tenter frame. The white, pure finished fabric has a count of 66 x 41 and a weight of 4 oz. per yard. This fabric is then passed through an impregnating solution containing 60 cubic centimeters of glyoxal solution (of 30.2% glyoxal content by weight), 3 grams of oxalic acid, 45 grams of water-dispersible urea formaldehyde condensation product known as P-364 Beckamine, and 6 grams of the quaternary ammonium salt, octa decyl oxymethyl pyridinium chloride per liter of solution. On a weight percentage basis this solution contains 2.25% glyoxal, 0.296% oxalic acid, 3.36% urea formaldehyde reaction product and 0.56% quaternary compound by weight. After the fabric is passed through this solution and is well wetted out, it is squeezed to remove excess solution and is then dried on a tenter frame in air at around 180° F. to dimensions before impregnating. The dried fabric is then cured in a tenter oven or loop dryer oven in circulating air at 280° F. for 8 minutes, after which it is soaped, rinsed and dried to the original pure finish fabric dimensions on a tenter frame. The resulting fabric is white, free from any odor, soft and resilient, with greatly improved resistance to shrinkage on washing, which effect is permanent to washing, and has improved resistance to creasing and crushing. A comparison of these properties of the untreated pure finish fabric and of the treated fabric is shown below. The table shows only the warp shrinkage. The filling shrinkage is always much lower in the untreated fabric, and is also satisfactorily controlled. The tensile strength and abrasion resistance of the fabric are not appreciably affected by the process.

## 10

lower in the untreated fabric, and is also satisfactorily controlled. The tensile strength and abrasion resistance of the fabric are not appreciably affected by the process.

*Shrinkage on washing, inches per yard*

[5 modified rayon washes—mild soap solution at 100°-120° F. for 30 min.]

| Washes.....    | Warp 1 | Warp 2 | Warp 3 | Warp 4 | Warp 5 |
|----------------|--------|--------|--------|--------|--------|
| Untreated..... | 6.10   | 6.53   | 7.13   | 7.03   | 7.23   |
| Treated.....   | 0      | .1     | 0      | .1     | .1     |

The process loss is 1.3 inches per yard in the warp.

*Crease resistance*

[Percentage recovery in one min. from 180° fold formed under standard conditions]

|                 | Per cent |
|-----------------|----------|
| Untreated ..... | 45       |
| Treated .....   | 75       |

## EXAMPLE 7

A plain weave, 100% spun viscose rayon fabric in the greige, made of 28/1 warp and 14/1 filling yarns of spun rayon viscose rayon staple fiber is desized, scoured and dried on a tenter frame. The white, pure finished fabric has a count of 66 x 41 and a weight of 4 oz. per yard. This fabric is then passed through an impregnating solution containing 60 cubic centimeters of glyoxal solution (of 30.2% glyoxal content by weight), 3 grams of oxalic acid, 45 grams of water-dispersible urea formaldehyde condensation product known as P-364 Beckamine, and 6 grams of the quaternary ammonium salt, octa decyl oxymethyl pyridinium chloride per liter of solution. On a weight percentage basis this solution contains 2.25% glyoxal, 0.296% oxalic acid, 3.36% urea formaldehyde reaction product and 0.56% quaternary compound by weight. After the fabric is passed through this solution and is well wetted out, it is squeezed to remove excess solution and is then dried on a tenter frame in air at around 180° F. to dimensions before impregnating. The dried fabric is then cured in a tenter oven or loop dryer oven in circulating air at 280° F. for 8 minutes, after which it is soaped, rinsed and dried to the original pure finish fabric dimensions on a tenter frame. The resulting fabric is white, free from any odor, soft and resilient, with greatly improved resistance to shrinkage on washing, which effect is permanent to washing, and has improved resistance to creasing and crushing. The fabric is found to be water-repellent and retains most of its water repellency through at least five launderings. A comparison of these properties of the untreated pure finish fabric and of the treated fabric is shown below. The table shows only the warp shrinkage. The filling shrinkage is always much lower in the untreated fabric, and is also satisfactorily controlled. The tensile strength and abrasion resistance of the fabric are not appreciably affected by the process.

*Shrinkage on washing, inches per yard*

[5 modified rayon washes—mild soap solution at 100°-120° F. for 30 min.]

| Washes.....    | Warp 1 | Warp 2 | Warp 3 | Warp 4 | Warp 5 |
|----------------|--------|--------|--------|--------|--------|
| Untreated..... | 6.10   | 6.53   | 7.13   | 7.03   | 7.23   |
| Treated.....   | 0      | .1     | 0      | .1     | .1     |

The process loss is 1.5 inches per yard in the warp.

*Crease resistance*

[Percentage recovery in one min. from a 180° fold formed under standard conditions]

|           | Per cent |
|-----------|----------|
| Untreated | 45       |
| Treated   | 95       |

As more particularly pointed out in the aforesaid application, it appears that the glyoxal treatment affects the individual fiber throughout its entire structure, causing a partial but incomplete conversion of the cellulose. Apparently the same action takes place when the glyoxal is employed in association with a resin.

It is our belief that when cellulose fibers are treated with a thermosetting resinous compound there is a definite reaction between the cellulose and the resinous material and that some further condensation of the resinous material with itself also takes place during the curing operation.

We base our belief (with reference to the auto-condensation of the resinous material) upon the fact that an increase in wet strength of the fabric is observed when compared with the results produced by reacting the cellulose material with glyoxal alone. Apparently the combined treatment of cellulose fibers with glyoxal and a resinous material is to produce a fiber consisting in part of a reaction product of cellulose and glyoxal and in part of a reaction product of cellulose and the resinous material, with the resinous material in a more highly condensed state after curing than it was originally. Whatever actually takes place in the cellulose fiber when subjected to the combined treatment with glyoxal and the thermosetting resin, it is certain that the physical characteristics of the fiber are thereby modified.

For ready comparison of the results obtained by the present invention with those obtained by prior usual methods of stabilization by the employment of resins alone, or by the use of glyoxal alone as described in the aforementioned application, reference may be had to the table shown in the drawing. In this table, column A indicates usual losses in scouring; column B the shrinkage of normal (untreated) fabric during five standard laundry washings; column 1 indicates the shrinkage losses in fabrics which have been treated with glyoxal alone; column 3 shows the losses in fabric treated with resin alone; and column 2 indicates losses in fabric treated with glyoxal together with a small amount of resinous condensation product.

In each of the columns B and 1 to 3 inclusive, there is a subcolumn headed "%5" and a second subcolumn headed "%1-5." The column headed "%5" represents the total shrinkage of the treated fabric in five modified washes without any process or working loss allowed. The column headed "%1-5" represents the difference in the measurements of the fabric between the first and fifth wash, or in other words, the progressive shrinkage between the first wash and the fifth wash. For example, if a fabric shows 3% shrinkage in the first wash and it still shows 3% shrinkage after the fifth wash, the %1-5 shrinkage is 0.

The table shows that the addition of a small quantity of resin to the glyoxal produces better stabilization than results from the use of glyoxal alone. For instance, the results obtained in column 2 are in most instances considerably better than those obtained in column 1.

The mixed process in which both glyoxal and resinous material are employed not only produces dimensional stability but also crush resistance. However, it is important to note that the crush resistance is apparently produced solely by the glyoxal since there is not sufficient resin to have any appreciable effect on crush resistance.

It will be observed that in no case is the quantity of resin employed in association with the glyoxal even as much as 50% of the resin required when resin alone is used for stabilization.

It is also to be emphasized, as indicated by the above specific examples, that the resin in association with the glyoxal not only produces dimensional stability but also crush resistance. However, the crush resistance must be attributed to the glyoxal since there is not sufficient resin to produce crush resistance, it being noted that for effective crush resistance it is necessary when using resin alone to employ even more than the 8% shown in column 6, in fact to employ 14% or more of the resin.

To illustrate the neutral effect of the resin upon crease resistance, when used in the small percentages of the present invention, a fabric like that of Example 1 above described was stabilized using two different formulae as follows:

1. 60 cc. of glyoxal (30.2%) per liter, 3 grams of oxalic acid per liter.

2. 60 cc. of glyoxal (30.2%) per liter, 45 grams of P-364 Beckamine (75% resin content) per liter, 3 grams of oxalic acid per liter.

The following table shows the wash stability results obtained with these two treatments, with a working loss of 1.4 inches.

*Warp shrinkage—5 modified washes*

| Washes           | 1   | 2   | 3   | 4   | 5   |
|------------------|-----|-----|-----|-----|-----|
| Untreated fabric | 6.1 | 6.5 | 7.1 | 7.0 | 7.2 |
| Treated fabric:  |     |     |     |     |     |
| 1.               | 1.1 | 1.2 | 1.3 | 1.4 | 1.4 |
| 2.               | 0   | 0   | 0   | .1  | .1  |

The following table shows the results with these same two treatments regarding tensile strength, crease resistance and abrasion resistance.

|           | Tensile strength |         |      |         | Crease resistance | Abrasion resistance (Taber) |  |  |
|-----------|------------------|---------|------|---------|-------------------|-----------------------------|--|--|
|           | Dry              |         | Wet  |         |                   |                             |  |  |
|           | Warp             | Filling | Warp | Filling |                   |                             |  |  |
| Untreated | 51               | 59      | 23   | 29      | 45                | 135 turns.                  |  |  |
| Treated:  |                  |         |      |         |                   |                             |  |  |
| 1.        | 37               | 40      | 23   | 21      | 85                | Satisfactory.               |  |  |
| 2.        | 46               | 50      | 26   | 28      | 85                | Do.                         |  |  |

Thus while the addition of the small quantity of resin in accordance with the present invention does improve shrinkage control or dimensional stability and in some cases may improve the finish of the fabric, it apparently contributes nothing substantial to the crush resistance of the fabric.

As indicated in the above specific examples, various types of resinous condensation product may be used, among them the reaction product of urea and formaldehyde, known as dimethylol urea. Among the other resinous materials which are useful for the purpose is P-364 Beckamine. This is a reaction product of urea and formaldehyde in which the reaction or condensation is carried to the point where the material no longer

forms a clear solution in water but actually forms an extremely fine dispersion. In fact, this material is film forming from water dispersion which is not the case with a dimethylol urea solution. The P-364 Beckamine is also very stable on storage for this type of material. A dimethylol urea solution is not stable on storage. The alkyl urea resinous condensation product is formed by the reaction of an alkyl substituted urea and formaldehyde simultaneously with the reaction of urea and formaldehyde so that the final material might be called a co-condensation product of urea and substituted urea with formaldehyde. The material is definitely film forming and produces a stable solution in water.

Another useful resin is Aerotex M3, a water-soluble reaction product of low molecular weight of melamine and formaldehyde. It is water-soluble and the solution is quite stable on storage. It appears to be film forming from water solution to a certain degree.

It is also to be observed as indicated in the above specific examples, that more than one resin may be used in association with the glyoxal in the treating bath, but in any event the total quantity of resinous material is quite low, in fact substantially less than one-half the amount of resinous material which would be required for stabilization if no glyoxal were employed. For best results it appears that substantially the same limiting quantities of glyoxal should be used as when glyoxal is employed alone, while the quantity of resinous material would appear to be within a range of from 1% to 5% of the solution by weight.

When it is desired to impart a soft hand or feel to the fabric a cation-active softener is added to the treating bath in an amount approximately 1% by weight of the bath.

The term "cation-active" as used in the present sense, simply means that the active part of the molecule in these compounds is the cation rather than the anion, as is usual with many of the present finishing agents and dyes. Most cation-active compounds may be considered as derived from ammonium hydroxide  $\text{NH}_4\text{OH}$  where one or more of the H's are replaced by complex organic radicals. One type includes the quaternary ammonium compounds. Some are relatively simple while others are extremely complex products containing nitrogenous bases, such as pyridine, quinoline, acridine replacing the H's in the  $\text{NH}_4$  group. The possibilities in new compounds of this type seem unlimited.

The empirical formula of the pyridinium compounds can be represented by



wherein

R stands for an alkyl radical containing not less than 8 C atoms.

The group N(tert) represents the molecule of a tertiary base such as trimethylamine or pyridine.

X represents the acidic radical, preferably of a weak acid as typified by acetic or formic.

#### Mode of synthesis

Heat together an acylamidomethylol compound, for instance stearoamidomethanol with a salt of pyridine corresponding to the final salt desired, for instance pyridine hydrochloride in an excess of the free base.

Reaction proceeds according to the following equation:



The above synthesis does not apply where the acid radical selected for X is the radical of a weak acid, for instance—acetic or formic. For weak acid as acetic



25

While certain examples have hereinabove been given as illustrative of the utility of this invention, we consider it to be applicable to a wide variety of textile materials including fibers, yarns and fabric of

(1) Regenerated cellulose

- 35 a—Viscose  
b—Cuprammonium  
c—Saponified acetate

(2) Cotton cellulose

(3) Mixtures—Major part cellulose

- 40 a—Viscose-acetate  
b—Viscose-alarac (casein)  
c—Viscose-soya bean protein  
d—Viscose-peanut protein  
e—Viscose-wool  
f—Viscose-cotton

45 (4) Spun and filament yarns.

It is to be understood that the above are merely by way of example and not by way of limitation, and that the invention is inclusive of all modifications and equivalents falling within the terms of the appended claims.

We claim:

1. The method of stabilizing regenerated cellulose textile material which comprises as steps impregnating the material with an aqueous glyoxal solution containing between 0.6% and 4.65% by weight of glyoxal, an acid catalyst and an amino-formaldehyde thermosetting resinous condensation product in amount between 1% and 5% of the solution by weight, removing the material from the solution, and baking the material at a temperature between 212° F. and 350° F.

2. The method of stabilizing textile fabric predominantly of yarns of regenerated cellulose which comprises as steps immersing the fabric in an aqueous solution containing glyoxal approximately in the amount of 0.6% to 4.65% by weight in the treating solution, an amino-formaldehyde thermosetting resinous condensation product in total amount between 1% and 5% by weight of the solution, and oxalic acid, expressing excess fluid, drying the fabric under tension and baking the fabric at a temperature between 212° F. and 350° F. for a period of between two minutes 70 and forty minutes.

15

3. The method of stabilizing textile fabric predominantly of yarns of viscose rayon which comprises as steps immersing said fabric in a water solution containing between 0.6% and 4.65% by weight of glyoxal, between 1% and 5% by weight of an amino-formaldehyde thermosetting resinous water-dispersible condensation product, and between 0.0125% and 0.40% acid catalyst by weight, until it is thoroughly wet, extracting excess liquid, drying the fabric, and baking the fabric to react the glyoxal with the cellulose of the yarn.

4. The method of stabilizing textile fabric predominantly of yarns of regenerated cellulose which comprises as steps immersing said fabric in an aqueous treating medium containing from 15 to 120 cc. of an approximately 30% glyoxal solution (30.2% glyoxal by weight) and from 20 to 50 grams of a water-dispersible urea-formaldehyde condensation product per liter of solution 20

16

and an acid catalyst, until it is thoroughly wet, drying the fabric, baking it at a temperature between 212° F. and 350° F. for a period of from two minutes to forty minutes, thereby to react the cellulose of the yarns with the glyoxal, and washing, rinsing and drying the fabric.

5. As a new article of manufacture, the product produced according to the method set forth in claim 1.

10. 6. As a new article of manufacture, the product produced according to the method set forth in claim 2.

15. 7. As a new article of manufacture, the product produced according to the method set forth in claim 3.

15. 8. As a new article of manufacture, the product produced according to the method set forth in claim 4.

EDWARD C. PFEFFER, JR.  
JACK EPELBERG.